

May 23, 1972

RYO ANDO ET AL

3,664,827

METHOD FOR REFINING MOLTEN IRON OR MOLTEN IRON ALLOYS

Filed April 22, 1969

2 Sheets-Sheet 1



May 23, 1972

RYO ANDO ET AL

3,664,827

METHOD FOR REFINING MOLTEN IRON OR MOLTEN IRON ALLOYS

Filed April 22, 1969

2 Sheets-Sheet 2

FIG. 2



## 1

3,664,827

### METHOD FOR REFINING MOLTEN IRON OR MOLTEN IRON ALLOYS

Ryo Ando and Tsutomu Fukushima, Kanagawa-ken, Japan, assignors to Nippon Kokan Kabushiki Kaisha, Tokyo, Japan

Filed Apr. 22, 1969, Ser. No. 818,283

Claims priority, application Japan, Apr. 24, 1968,  
43/27,062

Int. Cl. C21c 7/00, 7/04

U.S. CL. 75—51

3 Claims

#### ABSTRACT OF THE DISCLOSURE

Method for refining molten iron or molten iron alloys which comprises steps of adding a reactant and stirring the upper layer portion of said molten metal while blowing oxygen thereonto, and substantial inertia of movement and natural convection caused by pouring said molten metal into the ladle being utilized to enforce stirring effect in the ladle.

#### BACKGROUND OF THE INVENTION

This invention relates to a novel method and apparatus for refining molten iron or iron alloys and more particularly to a method and apparatus for rapidly removing impurities in molten pig iron, especially phosphorus and sulphur by causing it to react with oxygen and slag. Thus, this invention contemplates to readily remove such impurities as phosphorus, sulphur and chromium and the like while limiting to the minimum the variation of other components, especially carbon, by mechanically stirring only the upper layer portion of molten iron kept in a ladle by means of a stirring rod made of carbonaceous material or other refractory material while at the same time blowing oxygen onto the surface of the iron through a lance and by continuously charging a required quantity of reactant.

It is known that when refining molten pig iron with oxygen, the quantity of impurities generally decreases in the order of silicon and carbon, and that during the final stage of decarburization the quantity of phosphorus, chromium, etc., decreases. Thus, with oxygen, it is impossible to rapidly refine low phosphorus, high carbon steel. However, where a slag is prepared which is suitable to remove phosphorus and chromium at low temperature and the molten iron is caused to react with such a slag it is possible to remove phosphorus, chromium and the like in preference to decarburization. However, as shown by the following equation, the dephosphorization reaction generally requires supply of oxygen.



For example, to reduce the quantity of phosphorus from 0.2% to 0.05%, 1.93 kg. (1.35 Nm.<sup>3</sup>) of oxygen per ton of molten metal pig iron is required. In order to perform rapid refining operation, it is desirable to blow oxygen in the form of pure oxygen or of air onto the surface of the molten pig iron through a lance. In this case, however, the temperature of the surface portion of the molten iron with oxygen being blown thereinto increases extremely, thus causing easy decarburization. Accordingly, in such a case, it has been known in the art to cause slag, which is advantageous for dephosphorization reaction, to contact with the molten iron over as wide area as possible and over constantly renewed surface so as to enhance the movement of the molten iron to prevent excess rise in the temperature at the surface to which oxygen is blown and to bring the supplied oxygen into dephosphorization reaction as fast as possible.

## 2

Based on these considerations the shaking ladle method, rotor method and the like have been proposed. Further, in the steel manufacturing furnace, soft blow refining with a L.D. converter has been practiced by utilizing a portion of above described considerations. Of these the shaking ladle method involves imparting eccentric motion to a container of the molten pig iron or the ladle itself for the purpose of increasing the speed of movement of the molten pig iron and to increase the contact surface between the slag and the molten iron. Accordingly, splash of the slag and molten pig iron becomes excessive which requires an excessively large container so that practical use of this method is limited.

The rotor method and the like do not result in rapid and sufficient dephosphorization. Moreover, any of these methods requires additional process steps to the existing refining steps, so that they are difficult to practice.

The soft blow refining process with a L.D. converter requires a refining time twice as long as the ordinary refining time. In addition, even when the slag is sufficiently removed initially since a substantial quantity of slag remains adhered to the furnace body there is a problem that phosphorus is again entrained in the iron during the finishing refining step.

#### SUMMARY OF THE INVENTION

It is therefore an object of this invention to provide a novel method and apparatus capable of removing impurities, especially phosphorus and sulphur from molten iron or iron alloys without the accompanying various difficulties described above.

According to this invention, use is made of a considerable inertia and convection of the molten pig iron existing after pouring it into a ladle and the mechanical stirring is limited to the area receiving the blown oxygen and the area near the contact surface between the slag and the molten pig iron, or to only the upper layer portion of the molten pig iron. In addition, in order to minimize the splash, means are used to create a plurality of small stirring whirls or eddies. With this invention, even when a ladle is charged to about 80 to 90% of its normal capacity, it is possible to perform a satisfactory refining operation so that the invention is readily applicable to the existing molten iron transfer step. Briefly stated, the apparatus of this invention comprises a mechanism for stirring the upper layer portion of the molten pig iron, a mechanism for blowing oxygen onto the surface of the molten pig iron, and a mechanism for charging a reactant into a ladle containing the molten pig iron.

#### BRIEF DESCRIPTION OF THE DRAWING

Other features and objects of this invention, the mechanism and operation thereof can be more fully understood from the following detailed description when taken in conjunction with the accompanying drawing in which:

FIG. 1 is a plan view of the apparatus embodying this invention, and;

FIG. 2 shows a vertical sectional view of the apparatus shown in FIG. 1 in which the left hand half shows a section taken along a line IIa—IIa and the right hand half shows a section taken along a line IIb—IIb in FIG. 1.

#### DETAILED DESCRIPTION OF THE PREFERRED EMBODIMENT

Referring now to the accompanying drawing, a ladle for receiving molten pig iron and mounted on a suitable carriage is disposed substantially below the center of a treating table supporting frame 1. Stirring rods 3 of carbonaceous material or other suitable refractory material are arranged in the upper portion of the ladle 2. Stirring rods 3 are secured to a disc 5 at the lower end of a stirring shaft 4 so that when the shaft 4 is lowered, the

stirring rods 3 are immersed into the upper portion of the molten pig iron kept in the ladle. The stirring shaft 4 is connected to a swinging frame 7 provided with three radial arms 6 and the vertical movement of shaft 4 is effected by a motor 8 connected to the swinging frame 7 through a reduction gearing. At the lower side of the free end of each arm 6 is projected a stub shaft 9. A shaft 11 driven through a suitable transmission mechanism by a motor 10 mounted on the treating table supporting frame 1 is provided thereon and the stub shafts 9 and the shaft 11 are interconnected with suitable eccentricity, for example, of 150 mm. Accordingly, as the motor 10 is energized to drive the shaft through the transmission mechanism, the stub shaft 9 will be rotated about the axis of the shaft 11 with a radius corresponding to said eccentricity. In this manner, as the respective stub shafts 9 are rotated eccentrically about the axis 11, the axis of stirring shaft 4 will be moved along a circle through arms 6 and the swinging frame 7, thus imparting a circular motion to stirring rods 3 to effect stirring of the surface of the molten pig iron.

The oxygen blowing mechanism comprises water cooled lances suspended from a supporting structure 12 upstanding from the treating table supporting frame 1. The water cooled lances include a first lance 13 which extends through a guide 14. First lance 13 is vertically moved by a suspension wire 15 and is fixed to guide 14 by means of a handle 16. A second lance 13' which extends through a guide 14' secured to the stirring shaft 4, is vertically moved by a suspension wire 15' and is secured to the stirring shaft 4 by means of a handle 16'. In this example, the number of first lances 13 that are fixed to the treating table supporting frame is three whereas the number of second lances 13' secured to swinging shaft 4 is one. Oxygen is supplied to the treating table supporting frame 1 through a conduit 17, and distribution pipes 18 branched from the conduit 17 are connected to lances 13 and 13' via flexible pipes 19 to blow oxygen onto the upper surface of the molten pig iron through the lower ends of lances 13 and 13'.

The reactant charging device includes a bucket 20 suspended from a hoist 21 movable along a beam 22 on the treating table supporting frame 1. The bucket 20 operated by the hoist 21 is used to supply the reactant into a hopper 23 mounted on the treating table supporting frame. At the bottom of the hopper 23 an electromagnetic feeder 24 is provided to incorporate the reactant onto the surface of the molten pig iron in the ladle through a chute 25. Thus, proper adjustment of the electromagnetic feeder 24 assures positive and constant supply of the reactants.

As has been described hereinabove, this invention provides a refining apparatus for molten iron comprising a stirring mechanism, an oxygen blowing mechanism and a reactant charging mechanism wherein oxygen is blown upon the surface of the molten pig iron through lances 13 and 13' while the surface layer portion of the molten pig iron is stirred by the operation of a motor 10 and wherein the reactant is continuously charged while the molten iron is stirred and the oxygen is blown. Accordingly, since only the surface layer portion is stirred, the powder required for this purpose may be relatively small particles, thus reducing the cost of installation. In addition, it is possible to blow a large quantity of oxygen at high efficiencies. As the pressure of blowing oxygen is low, the slag forming agent may be in the form of small granules which not only increases the speed of forming the desired

slag but also enables readily adjustments of slag composition and temperature. Further it is possible to employ existing ladles without the necessity of changing the process steps.

Thus, this invention provides a novel method of refining iron and iron alloys which can readily and rapidly remove impurities therein and improve the efficiency of oxygen and reactants so that ordinary pig iron for cast iron and for steel manufacturing can be readily converted into pig iron of low phosphorus and sulphur content at very low cost. This also enables manufacture with converters species of steel which heretofore could be obtained only with electric furnaces. Similarly, when pig iron of low phosphorus and sulphur content or low silicon content is prepared with electric furnaces, it becomes possible to charge a large quantity of the pig iron into the electric furnace thus decreasing electric power and hence cost of the raw material. Further it is possible to increase the efficiency of steel manufacturing and the useful life of expensive refractories utilized in the furnace.

While the invention has been shown and described in terms of its preferred embodiments, it will be clear to those skilled in the art that many alterations and modifications may be made within the true spirit and scope of the invention. For example, it is possible to refine iron by the method of the present invention either simultaneously with or after desulphurization of pig iron. A plurality of lances for blowing oxygen may be provided aslant to the treating table supporting frame so as to blow oxygen from the upper corner of the ladle; and the location of said lance is not limited to that herein defined—i.e., in the axis of stirring shaft.

The decrease of carbon in the molten iron is small in the present refining method because the main object of the invention lies in the refining of impurities, and not in the decarburization of major carbon content.

What is claimed is:

1. In a method of refining molten iron or molten iron alloy wherein a reactant is added thereto and the molten metal or alloy is stirred, the improvement which comprises:

pouring said molten metal or alloy into a ladle, adding a predetermined quantity of a reactant proximate the surface of said molten metal or alloy, and stirring only said molten metal or alloy proximate the surface thereof while thereonto blowing oxygen.

2. The method of refining molten iron or molten iron alloy according to claim 1 wherein said reactant is added while there are substantial inertia of movement and natural convection caused by pouring said molten metal into said ladle.

3. The method of claim 1, wherein the molten metal is pig iron.

#### References Cited

##### UNITED STATES PATENTS

|           |         |         |         |
|-----------|---------|---------|---------|
| 2,110,066 | 3/1938  | Heuer   | 75—55 X |
| 2,290,961 | 7/1942  | Heuer   | 75—55 X |
| 2,397,737 | 4/1946  | Heuer   | 75—55   |
| 3,278,295 | 10/1966 | Ostberg | 75—61   |

L. DEWAYNE RUTLEDGE, Primary Examiner

J. E. LEGRU, Assistant Examiner

U.S. Cl. X.R.

65 75—50, 130